

# United States Patent [19]

Patterson

[11] 3,881,040

[45] Apr. 29, 1975

- [54] **METHOD FOR REMOVING EXCESS COATING MATERIAL FROM STRIP EDGES**
- [75] Inventor: **Robert W. Patterson**, Fairfield, Ala.
- [73] Assignee: **United States Steel Corporation**, Pittsburgh, Pa.
- [22] Filed: **Apr. 12, 1974**
- [21] Appl. No.: **460,320**

## Related U.S. Application Data

- [60] Continuation-in-part of Ser. No. 247,627, April 26, 1972, abandoned, which is a division of Ser. No. 117,987, Feb. 23, 1971, Pat. No. 3,685,484.
- [52] U.S. Cl. .... **427/349**; 118/63; 427/357
- [51] Int. Cl. .... **B05c 11/10**
- [58] Field of Search..... 117/102 M, 102 L, 102 R, 117/113, 114 A, 115; 118/63

[56]

## References Cited

### UNITED STATES PATENTS

3,480,469 11/1969 Shaffer ..... 117/102 M

Primary Examiner—Mayer Weinblatt  
Assistant Examiner—Edith L. Rollins

[57]

## ABSTRACT

A method for removing excess coating material from a coated strip in a slow speed coating operation in which the coating weight control is effected by an air knife. There is a tendency for the excess material to form "whiskers" at the strip edges. A wiper is positioned below the air knife and maintained in bearing relation against the strip edge to continuously scrape the excess material from the strip edge before it forms whiskers.

4 Claims, 2 Drawing Figures



FIG. 1.



PATENTED APR 29 1975

3,881,040

SHEET 2 OF 2

FIG. 2.



## METHOD FOR REMOVING EXCESS COATING MATERIAL FROM STRIP EDGES

This application is a continuation-in-part of application Ser. No. 247,627 filed Apr. 26, 1972, now abandoned which is a division of application Ser. No. 117,987 filed Feb. 23, 1971, now U.S. Pat. No. 3,685,484.

This invention relates to a method for removing excess coating material from the edges of coated strip produced in a slow speed coating operation in conjunction with air knives which are used for coating weight control.

Air knives are used to control the weight and distribution of a coating applied in hot dip coating operations, such as the galvanizing of steel strip. Air of a fluid under pressure is directed against the face of a coated substrate as it emerges vertically from a bath of molten coating material. This acts as a squeegee, removing excess coating material and causing it to flow back down the strip into the bath. The air jets may be horizontal but are generally inclined downwardly from 5° to 45° from the horizontal with about 20° to 25° being preferred for slow speed lines. Air knives, such as shown in my U.S. Pat. No. 3,406,656, tend to avoid build-up of the coating metal at the edges of the substrate when the substrate travels at relatively high speeds. However, when hot dip coating lines, such as a minimum spangle galvanizing line, are operated at speeds less than 150 feet per minute and air knives are used for coating control, whiskers are formed which adhere to each edge of the substrate. This is a particularly undesirable condition. Besides presenting a very unappealing appearance, whiskers cause safety and handling problems and cause coiling difficulties. Further, the cost of production is increased by loss of coating material as whiskers.

It is primary object of my invention to prevent the formation of dendritic structures or whiskers at the edges of coated substrates when air knives are used to control the coating weight in a slow speed dip-coating process.

I have found that by mechanically wiping the edge of a slow speed galvanizing line at the proper location, the formation of whiskers is avoided.

One embodiment of my invention is shown in the attached figures in which:

FIG. 1 is a diagrammatic elevation view of a hot dip coating apparatus with parts broken away.

FIG. 2 is an isometric view of a coated steel strip passing between air knives and mechanical edge wipers.

As shown in FIG. 1, a strip 10 enters a vessel 11 containing coating material 12 which in the galvanizing process is molten zinc, passes around a sinker roll 13 and moves upwardly between a pair of oppositely-disposed air knives 14 and is being contacted at its edges by wipers 16. The portion of the wiper in contact with the strip edge is A-shaped (FIG. 2). The cross bar 17 of the A actually contacts the strip while the legs 18 prevent the wiper from slipping off the strip edge. The wiper has an extended handle 20 which is adjustably positioned in tubular holder 21 and is retained therein by set screw 22. Affixed to holder 21 is an arm 24 which is carried by a support rod or axle 25 having integral retaining discs 26 at its ends. The edge wiper is positioned by placing the support rod 25 in a pair of toothed racks 27, only one off which is shown. A counterweight 28 is hung on a notch 29 in the arm to main-

tain sufficient bearing pressure of the wiper against the edge of the strip.

Unexpectedly, I found that the wiper is ineffective unless it contacts the strip at a point between about 1/2 inch and 4 inches below the point of impact of the air jet from the air knife. The optimum distance has proven to be about one inch below the point of impact of the air jet. The wiping must be accomplished while the zinc is still in the molten state and not after it becomes solidified. If the wiper is closer than 1/2 inch from the air jet, the air is turbulent and interferes with the wiping action. Also, the whiskers may already have formed and solidified. The following table shows the condition of the strip edge after cooling of the coating when the edge wiper is placed at various distances beneath the point of impact of the air jet against the strip.

TABLE I

| Distance<br>Beneath Jet Impact | Strip Edge Condition                 |
|--------------------------------|--------------------------------------|
| 0"                             | Unacceptable - Heavy whiskers        |
| 1/4"                           | Unacceptable - Light whiskers        |
| 1/2"                           | Acceptable                           |
| 1"                             | Excellent                            |
| 3"                             | Very good                            |
| 4"                             | Acceptable for sheet                 |
| 5"                             | Unacceptable for coils               |
| 5"                             | Unacceptable - Same as without wiper |

When the wiper is too far beneath the air jet, the molten zinc has not had time to move downward in relation to the strip, and the zinc climbs over the wiper, re-adhering to the strip edge. Further, the molten zinc which is being forced downwardly by the wiping action of the air knife spreads to the edges of the strip, causing additional edge buildup.

The position off the edge wiper may be adjusted vertically by use of set screw 22 and horizontally to accommodate various widths of strip by repositioning the support rod 25 in the toothed rack 27.

Edge wipers for removing excess coating material from strip edges are known. However, when an air knife is used, the vertical distance in which the wiper must operate is confined to about 4 inches, that being the distance between the bath and the air knife. Previous wipers, such as shown in LeCroy U.S. Pat. No. 3,536,038 do not have the necessary compactness to operate in this location. Shaffer U.S. Pat No. 3,480,469 shows a strip guide for use with an air knife, but his guide is not a wiper, as it is used to maintain a vacuum aspirator or wiper against the strip edge.

It can readily be seen from the foregoing that I have invented a method for preventing the formation of whiskers in slow speed hot dip coating lines in which the coating weight is controlled by use of an air knife.

I claim:

1. In a hot dip process for coating a strip by passing said strip, at a speed less than 150 ft./min., through a bath of coating material, removing said strip vertically from said bath, and controlling the coating thickness and distribution by directing a jet of fluid from a fluid nozzle against the face of the vertically-moving coated strip, the inclination of said jet being variable from normal to said strip to 45° downward, the improvement comprising preventing the formation of whiskers of coating material on the strip edge by contacting the edges of the strip by a mechanical wiper at a point be-

tween  $\frac{1}{2}$  and 4 inches beneath the point of impact of the fluid jet against said strip, maintaining said wiper in bearing relation against the edge of said strip, so as to continuously remove excess coating material from the strip edge and prevent such excess material from being contacted by the fluid emitted from said fluid nozzle.

2. An improvement according to claim 1 in which the

point of contact of said wiper is about 1 inch beneath said point of impact of said fluid jet.

3. An improvement according to claim 1 in which said strip is steel.

4. An improvement according to claim 1 in which said coating material is zinc.

\* \* \* \* \*

10

15

20

25

30

35

40

45

50

55

60

65